

## UNITED STATES PATENT OFFICE.

FRANK J. GROTE, JR., OF MERIDEN, CONNECTICUT, ASSIGNOR TO THE CONNECTICUT TELEPHONE & ELECTRIC COMPANY, INCORPORATED, OF MERIDEN, CONNECTICUT, A CORPORATION OF CONNECTICUT.

## MOLDABLE COMPOUND.

No Drawing.

Application filed November 10, 1922. Serial No. 600,016.

*To all whom it may concern:*

Be it known that I, FRANK J. GROTE, Jr., a citizen of the United States of America, residing at Meriden, Connecticut, have invented a new and useful Moldable Compound, of which the following is a specification.

My invention relates to a moldable compound and method of making the same. The compound is particularly adapted for molding in a cold state, that is, at atmospheric temperature though in some cases it may be found preferably or desirable to mold the compound while hot. The compound is especially adapted for the manufacture of parts such as electrical fittings.

It is the principal object of my invention to provide a compound which may be molded into articles which, when cured, will be relatively hard, will possess great mechanical strength and which will take a good polish.

It is a further object to provide a compound which will keep for a considerable length of time before molding without material deterioration, or undue setting or hardening.

It is a further object to provide a moldable compound which will be relatively inexpensive and with which rapid and uniform production in the molds may be attained.

The compound in its preferred form is composed of asbestos, boiled linseed oil, asphalt, and copal. In order to hasten the oxidation or drying of the compound an oxidizing agent or drier also may be added. The proportions of the various constituents may be varied between the approximate limits as follows: asbestos 84.2% to 72.4%; linseed oil 7.72% to 10.8%; asphalt 7.72% to 10.8%; and copal 36% to 6%. A preferably form of drier is a mixture of linseed oil and a metallic oxidizing agent, and the addition of a material quantity of such drier should be accompanied by a corresponding decrease of the proportion of linseed oil in order to keep the quantity of the latter within the desired limits. An example of a compound coming within the above limits, is asbestos 78%, linseed oil 8 1/2%, asphalt 9 1/2%, drier 1 1/3% and copal 2 2/3%.

In making the compound the ingredients

may be placed in a suitable container and heated together but I prefer to add the copal, preferably in the form of chips ground to 100 mesh, to the boiled linseed oil and heat the mixture to a temperature of, say 300° F. to 400° F. When the copal is dissolved the asphalt is added. If an oxidizing agent or so called drier is to be added, it is added to the above mixture preferably while hot and the mixture stirred until it is substantially uniform. The finely divided asbestos is put into a mixer and the hot liquid poured over it while the mixer is in operation, care being taken to distribute the liquid throughout the mass as nearly as possible. The mixer is run until the compound is substantially uniform throughout and until it is in a finely divided or powdered state. The mixing is likely to require several hours to secure the desired uniformity. After the mixing is continued for several hours, the compound will be dark in color and in finely divided form. The size of the particles will, of course, depend somewhat upon the proportions of the various ingredients and upon the length of time of mixing.

The ingredients when thoroughly mixed and powdered may be removed from the mixer and cured. This curing, which is really permitting oxidation, may be effected by exposing the material to the air for a time, but the time for thus curing the composition will be too great for economy since the process may take many days or even weeks with some compositions. In order to hasten production, the compound, on removal from the mixer, is preferably placed in a steam or other oven at a temperature of say 200° F. to 250° F. At this temperature the compound oxidizes fairly rapidly, and in twenty-four hours or so, depending upon the particular composition, the compound is ready for molding.

The function of the so called drier is to cause the compound to oxidize more rapidly, thus effecting a saving of time and greater production. It is desirable to oxidize the material as much as possible, but if almost completely oxidized, the compound will be difficult to mold and will require great pressure in the presses, and the material will not flow sufficiently freely in the molds to per-

mit the molding of delicate pieces, which require a rather free flowing of the material in the molds during the molding or pressing operation. The character of the piece 5 to be molded will, therefore, to a large extent, determine the degree of oxidation of the compound in the oven. After removal from the curing oven the material is screened and is then ready for molding.

10 While the compound may be molded as it comes from the mixer without material oxidation or curing, the results are not so satisfactory since the compound will often adhere to the molds and to prevent such adherence the molds must be lubricated before each piece is molded. When the compound 15 has been properly cured or oxidized, lubrication of the molds will be unnecessary and production will thus be increased materially.

The compound is molded in suitable molding presses, with or without metal inserts, and the molded articles are then cured, preferably by baking or heating in an oven, at 20 a temperature of say 400° F. until the articles are hard and of permanent character. The period of baking, of course, depends largely upon the size and character of the molded article and upon the particular composition and the length of time of the preliminary oxidizing. Good results may be obtained, with the compositions herein stated, by baking the molded articles for twenty-four to thirty hours.

35 The articles, after being baked or cured, are relatively hard, possess great mechanical strength, can be machined or drilled, and may be highly polished. In fact, the article as coming from the molds have a relatively 40 high polish. The articles are practically non-inflammable, and non-hygroscopic, retain their shape and are of permanent character.

45 While the ingredients of the compound as heretofore mentioned and the proportions heretofore mentioned are preferable, it should be understood that substitutions of other materials may be made, though at the present time I consider the proportions and 50 ingredients mentioned as the best. I consider that a part or all of the asbestos fibre might be replaced by other similar or inert material. It should likewise be noted that the boiled linseed oil might be replaced by 55 other drying or unsaturated oils. There are

other resins which might replace in whole or in part, the copal heretofore mentioned.

It might be stated that the so called drier herein mentioned is preferably boiled linseed oil with a metallic oxidizing agent therein. 60

It is preferable to use a small proportion of drier in order to hasten the curing of the compound, but I do not wish to be limited to the use of a drier, since the compound may be made without the use of drier, the advantage in the latter being that the curing is hastened and production thus increased. 65

The copal is preferably what is known as East India copal chips, and the addition of this material increases the strength of the 70 finished product materially. The asphaltic substance may be commercial Trinidad asphalt or similar material.

While I have described in detail a preferred composition of my compound and a 75 preferred method of making and using, I do not wish to be strictly limited thereto, since changes and modifications may be made within the scope of the appended claims.

I claim:

1. An article formed of a moldable composition which includes approximately, from 72.4% to 84.2% of inert material, from 7.72% to 10.8% of a drying oil, from 7.72% to 10.8% of an asphaltic substance, and from 0.36% to 6% of a resin of the copal type. 80

2. An article formed of a moldable composition which includes approximately, from 72.4% to 84.2% of inert material, from 7.72% to 10.8% of a drying oil with a drier, 90 from 7.72% to 10.8% of an asphaltic substance and from .36% to 6% of a resin of the copal type.

3. An article formed of a moldable composition which includes approximately, 78% 95 of an inert material, 8½% of a drying oil, 9½% of an asphaltic substance, 1½% of a drier, and 2½% of a resin of the copal type.

4. An article formed of a moldable composition which includes approximately, from 72.4% to 84.2% of asbestos, from 7.72% to 10.8% of linseed oil, from 7.72% to 10.8% of asphalt, and from 0.36% to 6% of copal. 100

5. An article formed of a moldable composition which includes approximately, 78% 105 of asbestos, 8½% of boiled linseed oil, 9½% of asphalt, 1½% of a drier, and 2½% of copal.

FRANK J. GROTON, JR.